

## UNITED STATES PATENT OFFICE

WILLIAM H. ALLEN, OF DETROIT, MICHIGAN; DOROTHEA ALLEN, EXECUTRIX OF SAID WILLIAM H. ALLEN, DECEASED, ASSIGNOR TO GEORGE EDWIN MAURER, OF PHILADELPHIA, PENNSYLVANIA

## METHOD OF TREATING LEATHER

No Drawing.

Application filed August 5, 1927. Serial No. 211,003.

The present invention relates to a method of treating leather and to the product produced thereby.

Heretofore in the production of leather from the skins of certain animals, the products are limited in their application, and, therefore their value, by reason of the fact that they are soft and spongy and of little strength and resistance to wear and distortion.

10 Among the objects of the present invention is to overcome such objections and to produce a leather from these same kinds of skins which has much greater "body", is 15 tough and strong and is capable of being used satisfactorily for purposes for which it was not before adapted.

The process consists in what might be called a "densifying" process, as examination 20 of the product indicates an apparent lessening of the intercellular spaces and a thickening of the cell walls with a very great increase in tensile strength, and involves a treatment preferably intermediate the tanning and finishing steps.

In carrying out the process, the preferred 25 method comprises placing the still wet skin from the tanning process, in a solution of a deliquescent salt that has no chemical affinity for the tanned skin, leaving the skin in said solution sufficiently long for the salt to dialyse into the membranes. After a sufficient time has elapsed usually from one to one and one half hours, the skin is by any 30 suitable method, such as rolling then taken from the solution, the excess water removed, and allowed to dry.

In the drying, the skin shrinks uniformly and considerably in length and breadth, that 40 is, in area, and generally increases somewhat in thickness. The decrease in area is permanent and may be as much as approximately one half, and, as such shrinkage is quite gradual, it may be halted at any desired point 45 by carrying out the next step at the desired time.

The next step consists in subjecting the shrunken skin to a washing operation to remove the salt. After thorough washing, the 50 skin is then finished in the usual manner,

such as by dyeing, fat-liquoring—dried and finished. While the preferred method involves the soaking of the skin in the solution of the treating salt, this step may also be carried out by sprinkling a solution of the salt upon the skin or the dry salt 55 sprinkled thereon and folded or rolled up in the wet skin.

The preferred treatment is with a 10 to 30% solution of calcium chloride but magnesium chloride may be substituted with good 60 results.

In those cases where the color produced will not be objectionable ferric chloride may also be used to produce the desired "densifying".

The action seems to be due to an abstraction of the last traces of uncombined water from the hide substance.

Further, either bark tanned or chrome 70 tanned skins may be treated in the process and these may be either with or without the naturally attached hair on them as the treatment does not in any way affect the hair except to thicken the fur by the reduction in 75 area of the skin. Also while the treatment may be applied to any kind of tanned skins, it is most beneficial for such skins as sheepskins or any that ordinarily are soft, spongy and of little strength.

The softer parts of cowhides such as the belly and sides may be lessened in area and increased in thickness and in tensile strength by said process and thus made suitable for 85 applications where heretofore only selected portions have been considered fit.

Now having described the invention and the preferred forms of embodiment thereof, it is to be understood that the said invention is to be limited not to the specific details 90 herein set forth but only by the scope of the claims which follow.

I claim:—

1. The process of treating tanned skins 95 of animals which comprises impregnating said skins with a salt inert to the tanned hide substance and capable of absorbing water, drying the impregnated skin and halting the shrinkage thereby produced at the 100

- desired point by washing out the salt, and subsequently finishing the product.
2. The process of treating tanned skins of animals which comprises impregnating said skins with calcium chloride, drying the impregnated skin and halting the shrinkage thereby produced at the desired point by washing out the salt, and subsequently finishing the product.
- 10 3. The process of treating tanned skins of animals which comprises soaking the wet skins from the tanning process in a solution of calcium chloride until thoroughly impregnated, drying said skins and thereby causing shrinkage, stopping said shrinkage at the desired point by washing out the calcium chloride, and subsequently finishing the so treated leather.

WILLIAM H. ALLEN.

20

25

30

35

40

45

50

55

60

65